

Nov. 7, 1961

E. J. SMITH ET AL

3,007,854

METHOD OF ELECTRODEPOSITING ALUMINUM ON A METAL BASE

Filed June 14, 1957

2 Sheets-Sheet 1



Nov. 7, 1961

E. J. SMITH ET AL

3,007,854

METHOD OF ELECTRODEPOSITING ALUMINUM ON A METAL BASE

Filed June 14, 1957

2 Sheets-Sheet 2



INVENTORS  
EDWIN J. SMITH  
MICHAEL G. VUCICH

BY *Stanley & O'Neil*

ATTORNEYS

1

3,007,854

**METHOD OF ELECTRODEPOSITING ALUMINUM ON A METAL BASE**

Edwin J. Smith, Steubenville, Ohio, and Michael G. Vucich, Bridgeville, Pa., assignors to National Steel Corporation, a corporation of Delaware

Filed June 14, 1957, Ser. No. 665,743

14 Claims. (Cl. 204—28)

This invention relates to an improved method of and 10 apparatus for the electrodeposition of aluminum on a metal base.

This application is a continuation-in-part of application Serial No. 512,734, filed June 2, 1955, and now abandoned, by Edwin J. Smith et al. for "Plating Apparatus and Method."

The present invention will be described and illustrated hereinafter with reference to the electrodeposition of aluminum on ferrous metal strip using a fused electrolyte containing predominant proportions of aluminum chloride. However, it will be apparent to those skilled in the art that the principles of this invention are applicable to other base metals, or forms of base metals, or coating metals, or other electrolytes presenting the problems solved by the invention.

A fused electrolyte composition having a free aluminum chloride content of approximately 75-85% by weight of the composition, with the remainder being sodium and/or potassium chloride, will produce good aluminum plate when plating ferrous metal strip. The above electrolyte composition may be either of the binary or ternary types, a satisfactory binary electrolyte composition being exemplified by a composition containing by weight 85% aluminum chloride and 15% sodium chloride; while a satisfactory ternary electrolyte may be exemplified by a composition containing by weight 80% aluminum chloride, 10% sodium chloride, and 10% potassium chloride. Although a fused electrolyte containing from 80-85% aluminum chloride produces objectionable visible fuming in the presence of water, an electrolyte containing more than 85% aluminum chloride fumes excessively and the plating results obtained are not improved by increasing the aluminum chloride above this value. However, if the aluminum chloride content of the fused electrolyte falls below about 75% by weight, poor plating results and such electrolyte compositions are not generally considered to be satisfactory.

The above mentioned visible fuming is a result of the reaction between the fused aluminum chloride and atmospheric water vapor, or water from some other source. The fumes thus produced are highly corrosive and if vented to the atmosphere they offer serious health hazards. The fumes also tend to corrode metallic apparatus with which they come in contact that is constructed of the usual materials of construction, thereby reducing its useful life at an uneconomic rate. For example, if a blower system is used for removing the fumes directly from the electroplating bath, the fumes are so corrosive that they attack the blower system and, after short periods of time, damage the same unless the materials of construction are non-corrosive relatively expensive metals or alloys.

It has been proposed to eliminate the fuming problem by sealing off the electroplating bath by means of a hood having entrance and exit slots, these slots being closed by flaps of resilient material which permitted movement of the strip therethrough while largely preventing escape of fumes from the electroplating bath. In such case, whether or not atmospheric air leaked into the hood in small amounts via the entrance and exit slots was not considered to be of great importance. However, applicants have discovered that even though the fuming problem is eliminated

2

by use of the slotted hood, after long periods of continuous plating a point is eventually reached where it is impossible to plate a satisfactory deposit of aluminum onto the strip. They discovered that these plating difficulties could be 5 corrected only by replacing the electrolyte with fresh electrolyte. In applicants' above-mentioned copending parent application, on the other hand, perfect hermetic sealing of the electrolyte bath surface and a conditioning of the strip are achieved by means of entrance and exit liquid seals through which the strip passes on entering and leaving the plating zone. The liquid seal type of sealing therefore eliminates the fuming problem and, even more important, eliminates the plating difficulties arising from contaminated electrolyte.

In both methods, namely, that using the liquid seals and that using the slotted hood, the strip to be plated was thoroughly dried prior to entry into the plating zone. Furthermore, the temperature of the electroplating bath in both cases was maintained well above the boiling point 20 of water. Despite the foregoing, applicants have discovered that water gets into the bath when using the slotted hood and acts to contaminate and interfere with plating. By detecting aluminum hydroxy chloride ( $AlCl_2OH$ ), aluminum dihydroxy chloride ( $AlCl(OH_2)_2$ ) or other 25 products of hydrolysis which are more acidic than the fused aluminum chloride electrolyte, applicants proved that despite the precautions associated with the slotted hood and despite the high temperature of the electroplating bath, water from some source gradually enters the 30 electroplating bath and causes its contamination.

Applicants have thus discovered that the entrance into the plating zone containing fused aluminum chloride electrolyte of even minute quantities of atmospheric air, or the presence on the strip surface of minute quantities of 35 free water, or combined water such as hydrated iron salts, or substances reacting under conditions present in the electroplating zone to form water, cause contamination of the electrolyte to a point where it is useless.

One result of this continued gradual contamination of 40 the electroplating bath with water in one or more of its various forms is that the concentration of the resulting products of hydrolysis builds up at the expense of free aluminum chloride, and since the concentration of free aluminum chloride is critical, eventually the electrolyte 45 is rendered useless and must be replaced. Another result of continued water contamination is an increase in the corrosivity of the electroplating bath due to the production of hydrochloric acid during hydrolysis of the aluminum chloride. Normally, the equipment in contact with the 50 electrolyte may be constructed of aluminum. However, the hydrochloric acid and other products of hydrolysis that are more acidic than the electrolyte quickly corrode the aluminum equipment and it must be replaced at frequent intervals. In addition, the hydrogen evolved presents 55 an appreciable explosive hazard. Still another difficulty resulting from water contamination of the electroplating bath is a build-up in the concentration of iron salts. It has been found that the deposition of aluminum is adversely affected when the concentration of iron exceeds about 0.02%. Since the hydrochloric acid produced 60 during hydrolysis of aluminum chloride also attacks the ferrous metal strip passing through the electroplating bath, the electroplating bath is soon contaminated with a sufficient amount of iron salts to cause difficulty and the contaminated electrolyte must be replaced if a high-quality 65 product is to be produced.

The above described water contamination of the electrolyte is particularly unexpected in view of the fact that the difficulties usually arising from visible fuming are 70 eliminated by the slotted hood type of sealing of the electroplating bath, taken with the high operating tem-

perature of the electroplating bath. It would be expected that this attempted isolation of the bath and the high operating temperatures would not allow any entry of water into the electroplating bath, particularly where the ferrous metal strip entering the electroplating bath is thoroughly dried. As mentioned above, where the liquid seal type of sealing is used, and the liquid of the liquid seal is maintained water-free, no contamination of the electroplating bath takes place due to the entrance of water.

The present invention therefore resides in the discovery that the fused aluminum chloride plating bath must be completely isolated from water, particularly from water vapor in atmospheric air, free water or combined water such as hydrated metal salts on the strip, and substances capable of reacting under the conditions present in the electroplating bath to form water and in the method and apparatus for accomplishing this purpose.

FIGURE 1 is a diagrammatic side elevational view partially in cross section of one embodiment of a continuous aluminum electroplating line in accordance with the present invention using the liquid seal type of sealing;

FIGURE 2 is a cross-sectional view taken along the line 2—2 of FIGURE 1 but omitting a showing of the strip, the rolls, and the electrodes for the purpose of clarity;

FIGURE 3 is a diagrammatic side elevational view, partially in cross section, of still another embodiment of a continuous electroplating line in accordance with the present invention, but using the slotted hood type of sealing; and

FIGURE 4 is a cross-sectional view taken along the line 4—4 of FIGURE 3 but omitting a showing of the strip, the sealing flaps, the rolls, and the electrodes for the purpose of clarity.

Referring now to the drawing and more particularly to FIGURES 1 and 2, a specific embodiment of the invention employing the liquid seal type of sealing will be first described. For the purpose of wet pretreatment of the strip prior to electrodeposition of aluminum, the strip 10 may be fed from coil 12 supported on coil support means 14 through cathodic cleaning tank 16, brushing and spraying apparatus 18, anodic pickling tank 20, brushing and spraying apparatus 22, heater 45 and unit 24, by means of a path established by rolls 26, 28, 30, 32, 34, 36, 38, 40, 42, 44, 46, 48 and 50. In cleaning tank 16, between rolls 26 and 28 the strip is made electro-negative by connecting the negative side of generator 52 (or any other suitable source of current) to conductor roll 26 and the positive side of generator 52 to anodes 54. A suitable cleaning medium for tank 16 has been found to be a heated "Orthosil" ( $Na_4SiO_4$ ) solution when employing a treating time of 10 to 15 seconds at a minimum current density of 35 amperes per square foot. Any other conventional cathodic cleaning solution employing an alkaline material of high conductivity, good wetting power and free-rinsing qualities normally used in the electrolytic cleaning of ferrous metal strip will, however, serve the purposes of this cleaning operation.

After leaving cleaning tank 16, the strip 10 passes through brushing and spraying apparatus 18 where it is contacted with rotary brushes 56 both before and after water washing from spray devices 58. This operation removes drag-out cleaning solution from tank 16 and mechanically scours the surface of the strip 10 to remove any loosened film on its surface. Squeegee rolls 32 and 34 remove surface water from the strip.

From brushing and spraying apparatus 18, the strip 10 passes over roll 36 and into anodic pickler 20. Between rolls 36 and 38 the strip is made electropositive by connecting the positive side of generator 60 (or any other suitable source of current) to conductor roll 36 and the negative side of generator 60 to cathodes 62. For the purpose of the anodic pickling operation occurring in tank 20, a suitable electrolyte has been found to be an aqueous sulfuric acid solution of a minimum con-

centration of 35% sulfuric acid when employing anodic pickling for two to three seconds at 80 to 100 amperes per square foot. However, for the purposes of this pickling operation, other conventional pickling solutions and treating conditions may be employed.

Upon leaving anodic pickler 20, the strip passes through brushing and spraying apparatus 22 where it is contacted by rotary brushes 64 both before and after contact by hot spray water from spray devices 66. This apparatus serves to remove drag-out pickle solution from the strip 10 as well as residual loosened oxide film, hydrated metal salts, etc. Squeegee rolls 42 and 44 serve to remove surface water from the strip 10 and the heat imparted to the strip by the hot spray water tends to cause it to flash dry.

After treatment of the ferrous metal strip in brushing and spraying apparatus 22, it passes through heater 45 and unit 24 over rolls 46, 48 and 50. In unit 24 the strip 10 is completely dried and may if desired be heated to an elevated temperature in a dry reducing atmosphere for the purpose of further conditioning the strip surface, or otherwise treated for the purpose of removing completely hydrated metal salts or other substances on the strip surface which are a source of water or which may react to produce water during subsequent passage of the strip through the electroplating line. Sealing flaps 70 are provided to reduce the loss of any treating gas employed within unit 24. For reasons to be explained hereinafter, it is important that the strip 10 leave unit 24 at the proper temperature for introduction into unit 72. In the event the strip is heated to a temperature higher than this requisite temperature, it is allowed to cool to a suitable temperature in section 74 of the unit 24, the heating and cooling portions of the unit being separated by a suitable baffle 76 provided with flaps 79. Once the strip has been thoroughly dried, the dry strip must not be subjected to any source of water while passing from the drying step to the electrolyte. It is preferred to surround the dry strip at all times with a dry medium such as a dry non-reactive gas, during passage from the drying step to the electroplating bath.

After wet pretreatment of the ferrous metal strip 10, it would be conventional in the art of electroplating ferrous metal with aluminum to subject the strip as a cathode to a fused aluminum plating electrolyte employing aluminum anodes. The resulting plate product, if treated in an electrolyte containing proper proportions of aluminum chloride, i.e., preferably about 80 to 85% aluminum chloride, and subjected to proper current conditions had a dense and adherent plated surface of aluminum. However, it was found that portions of the strip would exhibit a dark undercoating. This dark undercoating is objectionable from a standpoint of appearance to such an extent that the resulting plate would be less acceptable as a commercial product. Furthermore, this method of electroplating is subject to the many difficulties enumerated above in connection with water contamination and fuming of the electroplating bath.

In accordance with one important feature of the present invention, the problems resulting from water contamination and fuming of a fused electrolyte containing from about 80 to 85% aluminum chloride may be eliminated. The clue to the liquid seal means of eliminating this problem came from the discovery that a fused composition containing critical proportions of aluminum chloride and one or more of the other constituents of the fuming electrolyte, although not a satisfactory electrolyte for plating, is substantially non-fuming in the plating temperature range. By use of such a composition, water contamination and fuming of the fused electroplating bath are entirely prevented by eliminating contact between the electroplating bath and the atmosphere, and by completely removing prior to passing the strip into the electrolyte free water, hydrated metal salts, or other substances on the strip surface which are a source of water

or which will react to produce water under conditions present in the electroplating zone. Additionally, the electric current carrying characteristics of this non-fuming composition are such that it can provide a medium in which electrolytic surface treatment of the ferrous metal strip can take place which eliminates objectionable dark undercoating in the plated product. All this is accomplished by using the non-fuming composition as a liquid seal through which the strip passes on its way to and from the electroplating bath and at the same time, if desired, using the liquid of the seal on the entrance side of the electroplating bath as an electrolyte for an anodic treatment of the strip which in accordance with the present discovery eliminates all objectionable dark undercoating in the final plated product.

In a preferred embodiment of the present invention in which a ferrous metal strip is continuously plated with aluminum, the surface of the bath is enclosed and access to the bath is limited to strip inlet and outlet zones. Elimination of atmospheric contact with the electrolyte through the strip inlet and outlet zones in accordance with the liquid seal type of sealing is achieved by interposing a fused non-fuming composition of the type to be described hereinafter across the path of the inlet and outlet zones but out of contact with the fused aluminum plating electrolyte. The completely dried strip free of water or sources of water as above described is then fed into the electrolyte by passing it through a liquid seal, i.e., the interposed fused non-fuming composition, it is electroplated, and it subsequently emerges from the electrolyte through the exit zone by passage through the fused non-fuming composition interposed across its path. As will be explained more fully hereinafter, anodic treatment of the strip during its passage through the fused composition interposed across the inlet zone and prior to its entry into the electrolyte will condition the strip so as to assure a highly acceptable aluminum plated product.

More particularly and with reference to FIGURES 1 and 2 of the drawing, a fused electrolyte containing, for example, 82% aluminum chloride, 9% sodium chloride and 9% potassium chloride is contained in electroplating unit 80. A hood 82 of rectangular cross section and open at its lower end is positioned above electroplating unit 80 with its lower edges 84 below the level of the upper edges 86 of unit 80. Unit 72 which is to contain the non-fuming fused composition for the above mentioned purposes is shown constructed so it completely surrounds unit 80 while permitting the lower edges 84 of hood 82 to lie at a level below the level of the upper and outer edges 88 of unit 72. Upon filling unit 72 with a fused non-fuming composition of the present invention, such as 70% aluminum chloride, 15% potassium chloride and 15% sodium chloride, to a level above that of the lower edges 84 of hood 82 but below that of the upper edge 86 of the unit 80, atmospheric contact with the fuming electrolyte 78 is prevented. Furthermore, by extending the exit end of unit 24 below the surface of the non-fuming composition in unit 72, oxidation of strip 10 by atmosphere contact is prevented.

Electroplating unit 80 is provided with anodes 90 of high purity aluminum. These anodes are electrically connected to the positive side of a generator 92 (or some other source of electrical current) while the strip is made electronegative between rolls 94 and 96 by an electrical connection between roll 96 and the negative side of generator 92. Rolls 98, 100 and 103 serve to guide the strip through the fused non-fuming composition and into the electrolyte 78. Rolls 102 serve as squeegee rolls to remove drag-out composition from unit 72. It will be appreciated that a plurality of passes may be made through the electrolyte 78 for the purpose of electroplating with suitably arranged anodes for each pass. FIGURES 1 and 2 of the drawings illustrate a downward and upward pass only for the sake of simplicity.

Upon emerging from the electrolyte 78, the strip 10

passes through squeegee rolls 104 and is guided by rolls 106, 108 and 110 through the fused non-fuming composition of unit 72.

For the purpose of preventing heat leaks to the atmosphere, units 72 and 80 are positioned within unit 112 and insulating material or a heated medium such as oil are employed in the space 114. Additionally, and in order to maintain the electrolyte 78 and the non-fuming fused composition in unit 72 at the proper temperature, immersion heating may be employed.

In accordance with still another feature of the present invention, it has been found that the passage of the strip 10 through the non-fuming fused electrolyte 72 prior to electrodeposition of aluminum surface conditions the strip in a manner serving to lessen the dark undercoating condition often found to exist in the absence of such treatment. The extent of the surface conditioning obtained in the fused non-fuming composition is dependent in some degree on the time of treatment therein. Thus, the speed of the strip, the length of the path through the fused composition and the volume of non-fuming fused composition determines the effectiveness of this treatment. Still more satisfactory results may be obtained in the surface treatment by anodically treating the strip in the non-fuming composition. For the purpose of this anodic treatment, aluminum cathodes 116 are electrically connected to the negative side of generator 118 while the strip is made electropositive between rolls 50 and 98. Current densities of 25 to 50 amperes per square foot for 5 seconds have been found satisfactory for this treatment. Minimum current densities and time conditions are dictated by the extent of the surface condition being rectified. Maximum current densities and time conditions are dictated by the extent this treatment can be carried out without pitting the base metal to an extent which will interfere with the quality of the finished product.

Strip 10, after emergence from unit 72, has its drag-out losses reduced by the action of squeegee rolls 120 and then passes via rolls 110 and 122 into unit 124 where hot water sprays 126 serve to remove any excess material carried from the electroplating unit. The strip subsequently passes via rolls 128, 130 and 132 to coiling unit 134. During this passage, the strip may be heated in unit 136 for the purpose of assuring complete drying prior to coiling.

In accordance with the present invention those compositions which are suitable for use as a liquid seal in eliminating the water contamination and fuming problems associated with the electroplating electrolyte and/or providing a medium for treating the strip prior to electroplating in order to obtain improved results are those aluminum chloride containing compositions in which the aluminum chloride content is less than 70% by weight. The balance of this fused non-fuming composition is made up of at least one salt selected from the group consisting of sodium chloride and potassium chloride. In the case of a binary plating electrolyte such as 80 to 85% aluminum chloride and 20 to 15% sodium chloride, the preferred non-fuming fused composition of the present invention would consist of aluminum chloride and sodium chloride, the aluminum chloride content being less than 70% by weight. In the case of a ternary electrolyte such as one containing from 80 to 85% aluminum chloride and the balance sodium chloride and potassium chloride, the preferred fused non-fuming composition would consist of aluminum chloride, sodium chloride and potassium chloride, the aluminum chloride content being less than 70% by weight.

More specifically, the non-fuming compositions of the present invention comprise those compositions containing aluminum chloride and at least one salt selected from the group consisting of sodium chloride and potassium chloride in which the proportion of aluminum chloride is less than about 52 mol percent. When the mol percent of aluminum chloride is less than about 52%, the vapor

pressure of aluminum chloride at practical operating temperatures (below 400° F.) is not sufficient to permit fuming. At a preferred upper aluminum chloride proportion of not more than 50 mol percent, temperature appears to have no appreciable effect on fuming. This is thought to be, in the case of the binary non-fuming compositions, owing to the formation of the compound  $\text{NaAlCl}_4$  or  $\text{KAlCl}_4$ . In the case of the ternary electrolyte, a mixture of these compounds is apparently formed. In such cases, any excess sodium chloride or potassium chloride would be present as a free salt.

An important aspect of the present invention is the fact that the composition employed to eliminate the water contamination and fuming problems associated with the electrolyte contains or may contain substantially the same constituents as the electrolyte. Since this is true, drag-out losses on the strip from the non-fuming composition will not introduce undesired components into the electrolyte. Furthermore drag-out losses from the electrolyte introduced into the fused non-fuming composition as the strip passes through the latter will not contaminate the fused non-fuming composition with constituents other than those desired in a usable composition.

The fused non-fuming composition gradually becomes contaminated with undesirable products resulting from the hydrolysis of aluminum chloride, hydrated metal salts, etc., as it performs its function of preventing water contamination and fuming of the electrolyte. As a result, some provision must be made for maintaining the concentration of contaminates at a low level in order to prevent gradual contamination of the electrolyte through drag-out losses from the sealing bath. This may be accomplished by any one of a number of different methods such as by batch replacement of the contaminated sealing bath with a fresh fused non-fuming composition at intervals dictated by the rate of build-up in the concentration of contaminates, or by continuous or intermittent withdrawal of contaminated sealing composition and addition of fresh fused non-fuming composition to the sealing composition in quantities sufficient to maintain a low concentration of contaminates. An even more satisfactory method comprises combining either of the foregoing methods with continuously circulating the fused non-fuming composition to an enclosed storage tank filled with fused non-fuming composition and having a volume at least several times the volume of unit 72. Such continuous circulation is beneficial in that it assures a much more gradual build-up and better control over the concentration of contaminates.

It is desirable, as explained above, to employ a non-fuming sealing composition substantially free of water, products resulting from the hydrolysis of aluminum chloride, hydrated metal salts, iron salts, etc., and containing the same constituents as those present in the fuming electrolyte. This eliminates drag-out contamination of the electrolyte with constituents other than those already present. When employing a ternary electrolyte of aluminum chloride, potassium chloride and sodium chloride and a ternary non-fuming sealing composition of the same constituents, it is preferred to establish and maintain a weight ratio of potassium chloride to sodium chloride in the sealing composition identical with the weight ratio of potassium chloride to sodium chloride in the electrolyte. By doing this even though drag-out losses change the composition of the electrolyte slightly by reducing the aluminum chloride content and change the non-fuming composition by increasing its aluminum chloride content, the weight ratio of potassium chloride to sodium chloride remains the same in both the electrolyte and sealing compositions. As a result, when it becomes desirable to adjust the composition of either or both of these compositions so as to maintain proper operating conditions, there is no practical problem. In the case of the electrolyte, simple addition (either continuous or batch) of the proper amount of aluminum chloride will serve the pur-

pose. In the case of the non-fuming composition simple addition (either continuous or batch) of potassium chloride and sodium chloride in the same weight ratio as already present will serve the purpose. If this weight ratio were not initially the same in both the electrolyte and the sealing compositions, readjustment of the compositions during or between plating operations would be exceedingly complicated instead of a routine operational problem within the skill of the usual operating personnel.

The following exemplifies the meaning of identical weight ratios of potassium chloride to sodium chloride in the ternary electrolyte and non-fuming compositions. If the electrolyte initially consists of 84% aluminum chloride, 8% potassium chloride, and 8% sodium chloride (a 1:1 weight ratio of potassium chloride to sodium chloride), then a satisfactory non-fuming composition would be one containing 67% aluminum chloride, 16.5% potassium chloride, and 16.5% sodium chloride (also a 1:1 weight ratio of potassium chloride to sodium chloride). It is not however necessary for this feature of the invention that this weight ratio be a 1:1 ratio. Instead, another ratio such as a 4:1 ratio for the electrolyte would be suitable if the same weight ratio existed in the non-fuming sealing composition.

Since a change in the composition of the fused electrolyte will alter its melting or solidification point and since preferred conditions for electroplating are those at which the electrolyte composition is maintained at a relatively low temperature while still remaining in the fused state, it is impossible to state a range of preferred temperature for the electrolyte itself. It may be broadly stated that satisfactory plating will occur if the temperature of the electrolyte is maintained at some value lying between approximately 250° and 400° F. providing the electrolyte remains in the fused state. Thus, for example, a ternary composition containing 80% aluminum chloride, and 10% sodium chloride and 10% potassium chloride by weight was found to give good deposits at plating temperatures as low as 250° F. Assuming sufficient agitation, good deposits can be obtained at cathode efficiencies as high as 80% when employing current densities up to 150 amperes per square foot.

Referring now to FIGURES 3 and 4 of the drawing, which illustrate a specific embodiment of the invention employing the slotted hood type of sealing, the ferrous metal strip 210 after receiving a wet pretreatment in cathodic cleaning tank 16, brushing and spraying apparatus 18, anodic pickling tank 20 and brushing and spraying apparatus 22 identical with that previously described in connection with FIGURE 1, is shown passing under roll 227 and upwardly through heater 236 where it is heated sufficiently to completely evaporate any free water remaining on the strip surface. The heated ferrous metal strip 210 passes upwardly through strip conditioning unit 239 where the ferrous metal strip is thoroughly dried to remove any remaining traces of free water and then passes over rolls 237 and 238. If desired, the ferrous metal strip 210 may be treated within strip conditioning unit 239 in a reducing atmosphere or otherwise treated for the purpose of further conditioning the strip surface. Two pairs of suitable sealing flaps 240 and 241 are provided near the entrance and exit ends, respectively, of strip conditioning unit 239 to prevent undue loss of any dry gaseous treating agent which may be employed in strip conditioning unit 239, as well as aiding in preventing entry of atmospheric water vapor. The dry gaseous treating agent may be supplied to strip conditioning unit 239 by means of conduit 242 and withdrawn by means of conduit 243. The flow rate of dry gaseous treating agent to strip conditioning unit 239 via conduit 242 is controlled by valve 244, while the withdrawal rate via conduit 243 is controlled by means of valve 245. Any suitable dry gaseous treating agent may be employed in strip conditioning unit 239, depending upon the nature of the treatment desired. However, it is essential that the treat-

ment be such as to insure the surface of ferrous metal strip 210 being free of free water, combined water such as hydrated ferrous metal salts or substances reacting under conditions present in the electroplating zone to form water upon exit from strip conditioning unit 239. In addition, it is essential once the strip has been thoroughly dried and freed of all sources of water, that the dry strip not be subjected to any source of water while passing from the drying step to the electrolyte. It is preferred to surround the strip at all times with a dry medium, such as a dry, non-reactive gas, during passage from the drying step to the electroplating bath. In instances where a special conditioning treatment is not necessary, the gaseous treating agent may be dry air, dry nitrogen, dry carbon dioxide, dry argon, and the like. Usually, it is preferred that the gaseous treating agent be supplied to strip conditioning unit 239 at substantially atmospheric pressure.

The ferrous metal strip 210 passes downwardly from strip conditioning unit 239 into electroplating tank 246 containing fused electrolyte 247. The fused electrolyte 247 has a high aluminum chloride content such as for example 82% aluminum chloride, 9% sodium chloride and 9% potassium chloride, by weight, and fumes in the presence of water or water vapor under operating conditions. A hood 248 is positioned above electroplating tank 246, as best seen in FIG. 4. The exit end 207 of strip conditioning unit 239 extends downwardly a short distance through opening 286 in hood 248 and, similarly, the entrance end 208 of unit 268 extends downwardly a short distance through opening 287 in hood 248, thereby providing an entrance and an exit, respectively to electroplating tank 246 for ferrous metal strip 210. The hood 248 is joined to both strip conditioning unit 239 and unit 268 in air tight relationship, and since sealing flaps 241 and 271 are provided near ends 207 and 208, respectively, this combination of elements substantially seal off electrolyte 247 from the surrounding atmosphere. A dry gas such as dry nitrogen, dry carbon dioxide, dry argon, or dry air, is fed by means of conduit 249 into the space 285 within electroplating tank 246 above the level 284 of electrolyte 247 and the undersurface of hood 248. A valve 250 is provided in conduit 249 for the purpose of controlling the feed rate of dry gas fed to space 285.

Electroplating tank 246 is also provided with spaced pairs of anodes 251, 253, 254, 255, 256, 257, 258 and 259 of high purity aluminum. The ferrous metal strip 210 passes downwardly from roll 238, into fused electrolyte 247, and is subsequently passed between the spaced pairs of anodes 251, 253, 254, 255, 256, 257, 258 and 259 by means of a path established by rolls 252, 260, 261, 262, 263, 264 and 265. The spaced pairs of anodes 251, 253, 254, 255, 256, 257, 258 and 259 are electrically connected to the positive side of generator 266 (or other suitable source of current), while ferrous metal strip 210 is made electro-negative between contact rolls 238, 252, 261, 263 and 265 and the corresponding pairs of electrodes operably arranged with respect to each of the rolls by means comprising an electrical connection between each of the rolls and the negative side of generator 266. The ferrous metal strip 210 is electroplated with a coating of aluminum of desired thickness while within electroplating tank 246, with the electroplating conditions being substantially the same as described herein for FIGURES 1 and 2.

After passing under roll 265, the ferrous metal strip 210 passes upwardly through electrolyte 247 and after emerging therefrom passes between squeegee rolls 267, which tend to reduce the drag-out of electrolyte. The ferrous metal strip 210 continues to pass upwardly through unit 268, and then horizontally over rolls 269 and 270. A pair of sealing flaps 272 are provided at the exit end of unit 268 for the purpose of sealing off the exit and thereby allow a slight suction to be applied to unit 268 through exhaust conduit 273, if desired, as well as preventing the entry of atmospheric water vapor. The exhaust conduit 273 is provided with valve 274 for the purpose of con-

trolling exhaust of unit 268 in instances where unit 268 is exhausted. The plated ferrous metal strip 210, after passing over roll 270, passes from the exit end of unit 268 and is then washed with water and dried in the manner described for FIGURES 1 and 2.

For the purpose of minimizing loss of heat, electroplating tank 246 may be surrounded by an insulating material 283. Additionally, and in order to maintain the fused electrolyte 247 at the proper operating temperature, heating means (not shown) may be employed as conventional in the art. For example, immersion heating may be employed in the conventional manner, or preferably, the insulating material 283 may be spaced from the electroplating tank 246 and the electroplating tank 246 surrounded within the space thus formed between insulating material 283 and electroplating tank 246 by suitable heating means such as fin type strip heaters.

In accordance with the present invention, it is essential that the gas or gaseous mixture fed through conduit 249 be dry. The temperature of the entering gas may be at any suitable convenient temperature, such as room temperature. The pressure employed within space 285 may be any suitable convenient pressure, a pressure of substantially atmospheric pressure or slightly above having been found to be sufficient. Inasmuch as it is only necessary to replace the atmosphere within space 285 with a dry gas, and since a slight suction may be maintained, if desired, on strip conditioning unit 239 and unit 268 by means of exhaust conduits 243 and 273, respectively, thereby allowing the gas fed to space 285 together with any moisture or water content contained therein to more easily escape between the flexible sealing flaps 241 and 271 and ferrous metal strip 210, it is not usually necessary that the gas be supplied or the atmosphere within space 285 be maintained at a substantially elevated pressure. However, a pressure within space 285 above atmospheric pressure may be preferred in some instances for best results. The composition of the particular dry gas or dry gaseous mixture supplied to space 285 may vary widely. It is only necessary that the dry gas or gaseous mixture be substantially non-reactive under the conditions of operation of the electroplating line with the electrolyte 247, the ferrous metal strip 210, and the apparatus contacted by the gas or gaseous mixture. Suitable dry gases have been found to be nitrogen, argon, carbon dioxide, or even dry air, or mixtures thereof. However, best results are obtained when using a relatively heavy dry gas or gaseous mixture, with reference to air, such as carbon dioxide, argon, etc., rather than gases or gaseous mixtures lighter than air. The amount of dry gaseous treating agent supplied to space 285 will vary depending upon a number of factors such as the amount of contaminating moisture entering space 285, the volume of space 285, the rate of loss of dry gaseous treating agent, etc. When the volume of space 285 is 90 cubic feet, a dry gaseous treating agent feed rate of about 10-100 cubic feet per hour is generally sufficient under normal operating conditions. However, in every instance the feed rate of dry gaseous treating agent to space 285 is at least sufficient to provide a dry atmosphere therein, but larger quantities may be used. The gaseous treating agent may be supplied to space 285 intermittently but, preferably, it is supplied continuously for best results.

The provision of a dry gaseous atmosphere within space 285 has been found to be highly effective in controlling the gradual entry of water into the electroplating bath and the deleterious effects thereof. As a result, it is possible to continuously operate the slotted hood type of electroplating apparatus when using the method of the present invention over extended periods of time with substantially no water contamination or fuming of the electrolyte.

The foregoing detailed description and the following specific examples are for purposes of illustration only,

and are not intended as being limiting to the spirit or scope of the appended claims. All percentages appearing in the following examples are percent by weight.

*Example I*

A wet pretreated ferrous metal strip at a temperature of 375° F. and at a speed of 10 feet per minute is fed through plating apparatus similar to that illustrated in FIGURE 1, employing a fused non-fuming sealing composition for the purpose of eliminating water contamination and fuming of the electrolyte. The ferrous metal strip was completely free of free water, combined water such as hydrated metal salts, and substances reacting under conditions present in the electroplating zone to form water at the time of entering the electroplating zone.

The fused non-fuming composition is maintained at a temperature of 350° F. and contains 68.2% aluminum chloride, 15.9% potassium chloride and 15.9% sodium chloride. After passage through the inlet non-fuming composition the strip is introduced into an electrolyte which is maintained at a temperature of 325° F. and is of a composition comprising 80% aluminum chloride, 10% potassium chloride and 10% sodium chloride. Employing high purity aluminum anodes 10 feet in length, a 0.18 lb. per base box coating weight is obtained at current conditions of 42.5 amperes per square foot. Under these conditions, the cathode efficiency is 80%. After plating, the strip is fed from the electrolyte through the outlet zone having the non-fuming fused composition interposed across its path. During this operation, no fumes escape to the atmosphere and there is no indication of water contamination of the electrolyte even after an extended period of operation. The resulting plated product has a dense matte deposit of fine grain which is pleasing in appearance except for an occasional grayish appearance over small percentage areas of the strip. In addition, the coating is adherent, soft and ductile and can be mechanically brightened by light cold rolling.

*Example II*

The conditions of Example I are repeated except for the use of an anodic treatment in the non-fuming fused composition occupying the inlet zone. The anodic treatment employs high purity aluminum cathodes of about 2 foot length with current conditions of 40 amperes per square foot for 5 seconds.

The product of this example is identical with that of Example I except that the occasional grayish surface appearance over small percentage areas is eliminated with the result that upon brightening by light cold rolling or other means, the product is highly satisfactory in appearance.

*Example III*

The conditions of Example I are repeated except for the use of electroplating apparatus similar to that illustrated in FIGURE 3 employing the slotted hood type of sealing. Dry nitrogen is fed to space 285 at the rate of 72 cubic feet per hour, for the purpose of eliminating water contamination and fuming of the electrolyte. The volume within space 285 was about 90 cubic feet.

During this operation, no fumes escape to the atmosphere and there is no indication of water contamination of the electrolyte even after extended periods of operation. The product of this example is similar in appearance to that of Example II. However, the coating weight is considerably heavier due to the greater number of passes between the various pairs of electrodes.

What is claimed is:

1. In a method of electroplating an aluminum-containing coating on metal strip employing a fused body of electrolyte consisting essentially of aluminum chloride and alkali metal chloride, the steps comprising forming a substantially completely enclosed body of the electrolyte in an electroplating zone with a vapor space above at least

a portion of the body of electrolyte, treating the strip to remove completely free water, combined water and substances forming water under conditions present in the electroplating zone, passing the water-free treated strip through a seal into the body of electrolyte, preventing contact of moisture-containing atmospheric air with the body of electrolyte by passing water-free gas into the vapor space above the body of electrolyte in amounts sufficient to maintain a water-free atmosphere therein, the water-free gas being inert with respect to the electrolyte under the electroplating conditions and electroplating an aluminum-containing coating on the strip while in the body of electrolyte.

2. In a method of electroplating an aluminum-containing coating on metal strip employing a fused body of electrolyte consisting essentially of a predominant proportion of aluminum chloride and the remainder alkali metal chloride, the steps comprising contacting the strip surface with an aqueous media, forming a substantially completely enclosed body of the electrolyte in an electroplating zone with a vapor space above at least a portion of the body of electrolyte, treating the strip to remove completely free water, combined water and substances forming water under conditions present in the electroplating zone, passing the water-free treated strip through a seal into the body of electrolyte, surrounding the water-free treated strip with water-free gas while passing from the water removal step to the electrolyte, preventing contact of moisture-containing atmospheric air with the body of electrolyte by passing water-free gas into the vapor space in amounts sufficient to maintain a water-free atmosphere therein, the water-free gas being inert with respect to the electrolyte under the electroplating conditions and electroplating an aluminum-containing coating on the strip while in the body of electrolyte.

3. In a method of electroplating an aluminum-containing coating on metal strip employing a fused body of electrolyte consisting essentially of aluminum chloride and alkaline metal chloride, the steps comprising forming a substantially completely enclosed body of the electrolyte in an electroplating zone with a vapor space above at least a portion of the body of electrolyte, treating the strip to remove completely free water, combined water and substances forming water under conditions present in the electroplating zone, passing the water-free treated strip through a seal into the body of electrolyte, preventing contact of moisture-containing atmospheric air with the body of electrolyte by continuously passing water-free gas into the vapor space at a rate sufficient to maintain a water-free atmosphere therein, the water-free gas being inert with respect to the electrolyte under the electroplating conditions, continuously venting gas together with any water content from the vapor space above the body of electrolyte, and electroplating an aluminum-containing coating on the strip while in the body of electrolyte.

4. In a method of electroplating an aluminum-containing coating on metal strip employing a fused body of electrolyte consisting essentially of a predominant proportion of aluminum chloride and the remainder alkali metal chloride, the steps comprising contacting the strip surface with an aqueous media, forming a substantially completely enclosed body of the electrolyte in an electroplating zone with a vapor space above at least a portion of the body of electrolyte, treating the strip to remove completely free water, combined water and substances forming water under conditions present in the electroplating zone, passing the water-free treated strip through a seal into the body of electrolyte, surrounding the water-free treated strip with water-free gas while passing from the water removal step to the electrolyte, preventing contact of moisture-containing atmospheric air with the body of electrolyte by continuously passing water-free gas into the vapor space in amounts sufficient to maintain a water-free atmosphere therein, the water-free gas being inert

with respect to the electrolyte under the electroplating conditions, continuously venting gas together with any water content from the vapor space above the body of electrolyte, and electroplating an aluminum-containing coating on the strip while in the body of electrolyte.

5. In a method of electroplating an aluminum-containing coating on metal strip employing a fused body of electrolyte consisting essentially of aluminum chloride and alkali metal chloride, the steps comprising forming a substantially completely enclosed body of the electrolyte in an electroplating zone with a vapor space above at least a portion of the body of electrolyte, treating the strip to remove completely free water, combined water and substances forming water under conditions present in the electroplating zone, passing the water-free treated strip through a seal into the electroplating zone and through the body of electrolyte, preventing contact of moisture-containing atmospheric air with the body of electrolyte by passing water-free gas having a density greater than that of air into the vapor space in amounts sufficient to maintain a water-free atmosphere therein, the water-free gas being inert with respect to the electrolyte under electroplating conditions and electroplating an aluminum-containing coating on the strip passing through the body of electrolyte.

6. In a method of electroplating an aluminum-containing coating on metal strip employing a fused body of electrolyte consisting essentially of a predominant proportion of aluminum chloride and the remainder alkali metal chloride, the steps comprising treating the strip surface in an aqueous solution to remove foreign matter, thereafter washing the strip with water, forming a substantially completely enclosed body of the electrolyte in an electroplating zone with a vapor space above at least a portion of the body of electrolyte, treating the strip to remove completely free water, combined water and substances forming water under conditions present in the electroplating zone, passing the water-free treated strip through a seal into the electroplating zone and through the body of electrolyte, surrounding the water-free treated strip with water-free gas while passing from the water removal step to the electrolyte, preventing contact of moisture-containing atmospheric air with the body of electrolyte by passing water-free gas having a density greater than that of air into the vapor space in amounts sufficient to maintain a water-free atmosphere therein, the water free-gas being inert with respect to the electrolyte under the electroplating conditions and electroplating an aluminum-containing coating on the strip passing through the body of electrolyte.

7. In a method of electroplating an aluminum-containing coating on metal strip employing a fused body of electrolyte consisting essentially of aluminum chloride and alkali metal chloride, the steps comprising forming a substantially completely enclosed body of the electrolyte in an electroplating zone with a vapor space above at least a portion of the body of electrolyte, treating the strip to remove completely free water, combined water and substances forming water under conditions present in the electroplating zone, passing the water-free treated strip through a seal into the electroplating zone and through the body of electrolyte, preventing contact of moisture-containing atmospheric air with the body of electrolyte by continuously passing water-free gas having a density greater than that of air into the vapor space in amounts sufficient to maintain a water-free atmosphere therein, the water-free gas being inert with respect to the electrolyte under the electroplating conditions, continuously venting gas together with any water content from the vapor space above the body of electrolyte, and electroplating an aluminum-containing coating on the strip passing through the body of electrolyte.

8. In a method of electroplating an aluminum-containing coating on metal strip employing a fused body of electrolyte consisting essentially of a predominant pro-

portion of aluminum chloride and the remainder alkali metal chloride, the steps comprising treating the strip surface in an aqueous solution to remove foreign matter, thereafter washing the strip with water, forming a substantially completely enclosed body of the electrolyte in an electroplating zone with a vapor space above at least a portion of the body of electrolyte, treating the strip to remove completely free water, combined water and substances forming water under conditions present in the electroplating zone, passing the water-free treated strip through a seal into the electroplating zone and through the body of electrolyte, surrounding the water-free treated strip with water-free gas while passing from the water removal step to the electrolyte, preventing contact of moisture-containing atmospheric air with the body of electrolyte by continuously passing water-free gas having a density greater than that of air into the vapor space in amounts sufficient to maintain a water-free atmosphere therein, the water-free gas being inert with respect to the electrolyte under the electroplating conditions, continuously venting gas together with any water content from the vapor space above the body of electrolyte, and electroplating an aluminum-containing coating on the strip passing through the body of electrolyte.

9. In a method of electroplating an aluminum-containing coating on metal strip employing a fused body of electrolyte consisting essentially of at least about 75% by weight of aluminum chloride and the remainder alkali metal chloride, the steps comprising forming a substantially completely enclosed body of the electrolyte, treating the strip to remove completely free water, combined water and substances forming water under conditions present in the electroplating zone, providing an entrance to the enclosed body of electrolyte for the metal strip to be electroplated, interposing a liquid seal across the entrance to the body of electrolyte, the liquid seal being a non-fuming composition consisting essentially of not more than about 70 percent by weight aluminum chloride and the remainder alkali metal chloride passing the water-free treated strip through the liquid seal, strip entrance and the body of electrolyte, and electroplating an aluminum-containing coating on the strip passing through the body of electrolyte.

10. In a method of electroplating an aluminum-containing coating on metal strip employing a fused body of electrolyte consisting essentially of at least about 75% by weight of aluminum chloride and the remainder alkali metal chloride, the steps comprising treating the strip surface in an aqueous solution to remove foreign matter, thereafter washing the strip with water, forming a substantially completely enclosed body of the electrolyte, treating the strip to remove completely free water, combined water and substances forming water under conditions present in the electroplating zone, providing an entrance to the enclosed body of electrolyte for the metal strip to be electroplated, interposing a liquid seal across the entrance to the body of electrolyte, the liquid seal being a non-fuming composition consisting essentially of not more than about 70 percent by weight aluminum chloride and the remainder alkali metal chloride, passing the water-free treated strip through the liquid seal, strip entrance and the body of electrolyte, surrounding the water-free treated strip with water-free gas while passing from the water removal step to the liquid seal, and electroplating an aluminum-containing coating on the strip passing through the body of electrolyte.

11. In a method of electroplating an aluminum-containing coating on ferrous metal strip employing a fused body of electrolyte consisting essentially of at least about 75% by weight of aluminum chloride and the remainder alkali metal chloride, the steps comprising forming a substantially completely enclosed body of the electrolyte, treating the strip to remove completely free water, combined water and substances forming water under conditions present in the electroplating zone, providing an

entrance to the enclosed body of electrolyte for the ferrous metal strip to be electroplated, interposing a liquid seal across the entrance to the body of electrolyte, the liquid seal being a non-fuming composition consisting essentially of not more than about 70 percent by weight aluminum chloride and the remainder alkali metal chloride, maintaining the liquid seal substantially free of free water, combined water and substances forming water under conditions present in the electroplating zone by continuously withdrawing contaminated liquid sealing composition and supplying water-free liquid sealing composition, passing the water-free treated strip through the liquid seal, strip entrance and the body of electrolyte, and electroplating an aluminum-containing coating on the strip passing through the body of electrolyte.

12. In a method of electroplating an aluminum-containing coating on ferrous metal strip employing a fused body of electrolyte consisting essentially of at least about 75% by weight of aluminum chloride and the remainder alkali metal chloride, the steps comprising treating the strip surface in an aqueous solution to remove foreign matter, thereafter washing the strip with water, forming a substantially completely enclosed body of the electrolyte, treating the strip to remove completely free water, combined water and substances forming water under conditions present in the electroplating zone, providing an entrance to the enclosed body of electrolyte for the ferrous metal strip to be electroplated, interposing a liquid seal across the entrance to the body of electrolyte, the liquid seal being a non-fuming composition consisting essentially of not more than about 70 percent by weight aluminum chloride and the remainder alkali metal chloride, maintaining the liquid seal substantially free of free water, combined water and substances forming water under conditions present in the electroplating zone by continuously withdrawing contaminated liquid sealing composition and supplying water-free liquid sealing composition, passing the water-free treated strip through the liquid seal, strip entrance and the body of electrolyte, surrounding the water-free treated strip with water-free gas while passing from the water removal step to the liquid seal, and electroplating an aluminum-containing coating on the strip passing through the body of electrolyte.

13. In a method of electroplating an aluminum-containing coating on ferrous metal strip employing a fused body of electrolyte consisting essentially of at least about 75% by weight of aluminum chloride and the remainder alkali metal chloride, the steps comprising forming a substantially completely enclosed body of the electrolyte, treating the strip to remove completely free water, combined water and substances forming water under conditions present in the electroplating zone, providing an entrance to the enclosed body of electrolyte for the ferrous metal strip to be electroplated, interposing a liquid seal across the entrance to the body of electrolyte, the liquid seal being a non-fuming composition consisting essentially of not more than about 70 percent by weight aluminum chloride and the remainder alkali metal chloride maintaining the liquid seal substantially free of free water, combined water and substances forming water in the electroplating zone by replacing at least a portion of

contaminated liquid sealing composition with wafer-free liquid sealing composition, passing the water-free treated strip through the liquid seal, strip entrance and the body of electrolyte, surrounding the water-free treated strip with water-free gas while passing from the water removal step to the liquid seal, and electroplating an aluminum-containing coating on the strip passing through the body of electrolyte.

14. In a method of electroplating an aluminum-containing coating on ferrous metal strip employing a fused body of electrolyte consisting essentially of at least about 75% by weight of aluminum chloride and the remainder alkali metal chloride, the steps comprising treating the strip surface in an aqueous solution to remove foreign matter, thereafter washing the strip with water, forming a substantially completely enclosed body of the electrolyte, treating the strip to remove completely free water, combined water and substances forming water under conditions present in the electroplating zone, providing an entrance to the enclosed body of electrolyte for the ferrous metal strip to be electroplated, interposing a liquid seal across the entrance to the body of electrolyte, the liquid seal being a non-fuming composition consisting essentially of not more than about 70 percent by weight aluminum chloride and remainder alkali metal chloride maintaining the liquid seal substantially free of free water, combined water and substances forming water in the electroplating zone by replacing at least a portion of the contaminated liquid sealing composition with water-free liquid sealing composition, passing the water-free treated strip through the liquid seal, strip entrance and the body of electrolyte, surrounding the water-free treated strip with water-free gas while passing from the water removal step to the liquid seal, and electroplating an aluminum-containing coating on the strip passing through the body of electrolyte.

**References Cited in the file of this patent**

UNITED STATES PATENTS

|           |                 |                |
|-----------|-----------------|----------------|
| 1,004,673 | Monnot          | Oct. 3, 1911   |
| 1,068,411 | Chubb           | July 29, 1913  |
| 1,069,151 | Loewenthal      | Aug. 5, 1913   |
| 1,426,683 | Stalhane et al. | Aug. 22, 1922  |
| 1,488,553 | Peacock         | Apr. 1, 1924   |
| 1,927,772 | Chittum         | Sept. 19, 1933 |
| 1,942,025 | Frost           | Jan. 2, 1934   |
| 2,111,826 | Waltman et al.  | Mar. 22, 1938  |
| 2,332,978 | Ahern           | Oct. 26, 1943  |
| 2,370,973 | Lang            | Mar. 6, 1945   |
| 2,375,434 | Moise et al.    | May 8, 1945    |
| 2,418,088 | Nachtman        | Mar. 25, 1947  |
| 2,463,412 | Nachtman        | Mar. 1, 1949   |
| 2,643,975 | Neish           | June 30, 1953  |
| 2,699,415 | Nachtman        | Jan. 11, 1955  |

## FOREIGN PATENTS

484.014 Great Britain ----- Apr. 29, 1938

#### OTHER REFERENCES

Transactions of the Electrochemical Society, vol. 91, 1947, pages 203-219.